

Jan. 15, 1935.

H. SCOTT

1,987,714

HIGH TEMPERATURE THERMOSTATIC METAL

Filed Sept. 22, 1931



WITNESSES:  
Fred. G. Williams  
N. M. Biebel

INVENTOR  
Howard Scott  
BY  
Richard O. Marvine  
ATTORNEY

## UNITED STATES PATENT OFFICE

1,987,714

## HIGH TEMPERATURE THERMOSTATIC METAL

Howard Scott, Wilkinsburg, Pa., assignor to Westinghouse Electric & Manufacturing Company, a corporation of Pennsylvania

Application September 22, 1931, Serial No. 564,268

2 Claims. (Cl. 297—15)

My invention relates to thermally actuatable devices and particularly to bimetal thermostatic members.

Among the objects of my invention are the following: To provide a bimetal combination of two alloys of different temperature expansivities that shall have of the same order of hardness; to provide a high expansion component in a bimetal element that shall be ductile and that shall not have excessive hardness; to provide a bimetal combination that shall have such characteristics as to the relative hardness of the two components as will permit of fabricating the same relatively easily; to provide a bimetal element that shall have a relatively large coefficient of deflection with a predetermined change of temperature.

In practicing my invention I provide a bimetal element made up of two iron-base alloys, the high expansion component being a manganese-iron alloy having over 23% of manganese, while the low expansion component is a nickel-iron alloy with which may be mixed an appreciable percentage of cobalt. The two components of such a bimetal element may be operatively associated with each other in any desired manner usually practiced in this art.

The single figure of the drawing illustrates a bimetal strip or bar embodying my invention and shown in section.

In my Patent No. 1,671,491, I have disclosed and claimed a high-expansion component for a bimetal element that includes specifically an alloy of iron embodying not over 30% of manganese, which is operatively associated with a nickel-iron alloy containing up to or approximately 45% nickel. I have found that a bimetal element of the kind disclosed and claimed in this patent has desirable properties for use at temperatures having an average value of about 300° C. I have also found, however, that a bimetal combination of this kind, and particularly the high-expansion component thereof, suffers from a lack of ductility and is excessively hard, so that the fabrication

of a bimetal element of these alloys is relatively hard to accomplish and is, therefore, somewhat expensive.

Further experimental work along this line has indicated that the lack of ductility and the excessive hardness of the alloy including up to 25% of manganese can be overcome by the use of relatively larger manganese contents, and I have found it possible to use up to substantially 36% manganese, which is a greater percentage than would theoretically have seemed desirable.

One of the results accompanying the use of a higher percentage of manganese is that the temperature at which its expansivity changes rapidly from a low value to a high value, is increased. The temperature coefficient of expansion is, however, not changed appreciably from that of the alloy containing not over 25% of manganese above about 200° C.

If a higher deflection is desired at the lower temperatures, I may obtain the same by adding an alloying element of the order of 5%, or less, either singly or in combination, of nickel, copper, cobalt, chromium, silicon, molybdenum, or tungsten, to the iron-base alloy containing 23% to 36% of manganese, without serious loss in ductility. It may be desirable to maintain the combined percentage of manganese and one or a combination of the above-enumerated metals so as not to materially exceed 36%; that is, when substantially 5% of one or of a combination of the above-enumerated seven metals is used, the percentage content of manganese should not exceed 31% or 32%. This composition is set forth in combination VI of Table I where the five percent of added elements is to be considered as including a group consisting of these metals used singly or in combination.

The single figure of the drawing illustrates a strip or bar of bimetal in which the high-expansion component 11 is a manganese-iron alloy embodying the composition hereinafter set forth in Table I, while component 12 is a nickel-cobalt-

45

TABLE I  
High expansion component

50

|     | Manganese           | Carbon                | Silicon               | Added elements    | Remainder iron |
|-----|---------------------|-----------------------|-----------------------|-------------------|----------------|
| I   | Percent<br>28 to 36 | Percent<br>.05 to .30 | Percent<br>.05 to 1.0 | Percent<br>0 to 2 | Do.            |
| II  | 30 to 33            | .05 to .30            | .05 to 1.0            | 0 to 2            | Do.            |
| III | 30.5                | .15                   | .17                   | 0 to 1            | Do.            |
| IV  | 28 to 36            | .05 to .30            | .05 to 1.0            | 0 to 1            | Do.            |
| V   | 26 to 36            | .05 to .30            | .05 to 1.0            | 0 to 2            | Do.            |
| VI  | 23 to 31            | .05 to .30            | .05 to 1.0            | 1 to 5            | Do.            |

55

45

50

55

iron alloy which may be made up of any one of hereinbefore stated, the coefficient of deflection of the combinations hereinbelow shown in Table II, can be increased somewhat by the addition of an

TABLE II  
Low expansion component

5

5

10

10

|   | Nickel              | Cobalt               | Manganese                    | Silicon                           | Added elements              | Remainder iron |
|---|---------------------|----------------------|------------------------------|-----------------------------------|-----------------------------|----------------|
| A | Percent<br>25 to 50 | Percent<br>5<br>15.5 | Percent<br>.05 to 1.0<br>.22 | Percent<br>.05 to .5<br>.05 to .5 | Percent<br>0 to 1<br>0 to 1 | Do.            |
| B | 29.8                | 20                   | 3 to 32                      | .05 to 1                          | 0 to 2                      | Do.            |
| C | 26 to 32            | 3 to 20              | .1 to 2                      | .05 to .5                         | 0 to 2                      | Do.            |
| D | 35 to 50            | .1 to 2              | .05 to 1                     | .05 to .5                         | 0 to 2                      | Do.            |
| E | 45.2                | .1 to 2              | .06 to .53                   | .01 to .07                        | 0 to 1                      | Do.            |

15

15

It may be noted from Table I, that the range of percentage of manganese is from 23% to 36% with incidental metallic constituents not over 1% or 2%, the remainder being iron and an alloying element of not over 5% of copper, cobalt, chromium, nickel, silicon, molybdenum, or tungsten, either singly or in any desired combination. I have found it possible also to use substantially 30.5% of manganese, .15% of carbon, .17% silicon, less than 1% of incidental constituents with the remainder being iron and obtain substantially the same results as to ductility and hardness. By the incidental constituents, I mean the usual small quantities of impurities of one kind and another which are usually found to be present in an alloy or metal and which are of no particular effect as regards the particular characteristics which it is desired that the alloy or metal shall have.

Referring to the low expansion component set forth in Table II, it may be noted that I prefer to use more than 25% of nickel and may even use up to 50% of nickel, in combination with cobalt varying from 3% to 20%, from .05 to 1% of manganese, from .01% to .5% of silicon, from a trace to 2% of incidental constituents, the remainder being iron or steel.

By virtue of the lower hardness and higher ductility of the higher-manganese, iron-base alloys, as compared to such alloys having about 23% of manganese, bimetal elements made from the former, in combination with a low-expansion nickel-steel, may be fabricated, as by being welded or fused one to another, relatively easily, and may then be much more easily rolled, either cold or hot, (than bimetal elements using the 23 percent manganese steel) to the desired degree of thickness. The bimetal element or slab thus acts, in general, as a single metal element or slab, that is, the initial relative thicknesses of the two components will remain the same no matter how thin the strip or bar may be rolled. It is usually desirable to have the two components of equal thickness and I have found no trouble in obtaining a thickness of .01 inch for each of the two components when a thickness of the bimetal element of .02 inch was desired.

I have found that a bimetal element of this kind will have a relatively high deflection coefficient for a given change of temperature and will operate without loss of mechanical strength at a temperature well above 300° C. and as was

alloying element which may be either one or a combination of metals hereinbefore enumerated, all of which have relatively high temperature expansivities, the amount or percentage of the alloying element being relatively small but very effective.

The difference in expansivities of the two components has been found to be not more than  $12.0 \times 10^{-6}$  per °C. at 100° C. and greater than  $15.0 \times 10^{-6}$  per °C. at 300° C.

Various modifications may be made in my invention without departing from the spirit and scope thereof, and I desire, therefore, that only such limitations shall be placed thereon as are imposed by the prior art or are set forth in the appended claims.

I claim as my invention:

1. A bimetal element including two cooperating components having different temperature expansivities, the high expansion component being an alloy including from twenty-six to thirty-six percent of manganese, between one tenth percent to one percent of incidental constituents, from one to five percent of any one of the following or any combination thereof; copper, cobalt, chromium, nickel, silicon, molybdenum, tungsten, the remainder being principally iron, the low expansion component being an alloy including between twenty-five to fifty percent nickel, approximately fifteen percent cobalt, between one tenth percent and one percent incidental constituents, the remainder being principally iron.

2. A bimetal element including two cooperating components having different temperature expansivities, the high expansion component being an alloy including substantially thirty and one half percent of manganese, approximately fifteen hundredths percent of carbon, approximately seventeen hundredths percent of silicon, between one tenth and one percent of incidental constituents, between one and five percent of an alloying element from a group consisting of copper, cobalt, chromium, nickel, silicon, molybdenum, tungsten, the remainder being mainly iron, the low-expansion component being an alloy including twenty-nine and eight tenths percent of nickel, approximately fifteen percent of cobalt, approximately twenty-two hundredths percent of manganese, between one tenth and one percent of incidental constituents, the remainder being principally iron.

HOWARD SCOTT.